

## UNITED STATES PATENT OFFICE

ALFRED FISCHESSER, OF FRANKFORT-ON-THE-MAIN-FECHENHEIM, GERMANY, AS  
SIGNOR TO GENERAL ANILINE WORKS, INC., OF NEW YORK, N. Y., A CORPORATION  
OF DELAWARE

## DYEING ANIMAL FIBERS

No Drawing. Application filed August 4, 1930, Serial No. 473,124, and in Germany September 2, 1929.

My present invention relates to a process of dyeing animal fibers in the cold with leuco-ester salts of vat dyestuffs.

Leuco-ester salts of vat dyestuffs have hitherto been brought onto the animal fiber at elevated temperature and in an acid medium and the dyestuff developed by an after-treatment with an oxidizing agent.

10 In accordance with the present invention leuco-ester salts of vat dyestuffs can be fixed on the animal fiber also in an alkaline medium in the presence of a reducing agent.

15 It is a surprising fact that this process does not require an elevated temperature but takes place already at room temperature. In comparison with the hitherto usual dyeing processes it shows several important advantages. It allows mixed shades to be produced easily by suitable combinations. Furthermore, the material can be partially coated with fat, wax or other mechanical resist which in consequence of the low temperature prevailing suffers no injury during the following fixation of the ester-salt. In this manner white and colored batic-effects are produced on a colored ground and exhibit a clearness and beauty hitherto not obtainable 25 by means of leuco-ester salts of vat dyestuffs.

30 The present process may also be applied to mixed fabrics containing animal fibers.

In order to further illustrate my invention the following examples are given, the parts 35 being by weight and all temperatures in centigrade degrees, but it is however to be understood, that my invention is not limited to the particular products nor reacting conditions mentioned therein:—

## Example 1

Bleached wool is partially coated with one 45 of the customary wax resists (for instance

beeswax) and then treated with the following mixture:

|                                                                               |    |
|-------------------------------------------------------------------------------|----|
| 10 parts of the sulfuric acid ester-salt of leuco-5.7.5'-trichloro-indigo,    | 50 |
| 950 parts of lukewarm water,                                                  |    |
| 10 parts of ethylene-thiodiglycol,                                            |    |
| 10 parts of the sodium salt of benzyl-sulfanilic acid,                        |    |
| 10 parts of potassium carbonate,                                              |    |
| 10 parts of formaldehyde-sulfoxylate (which may be replaced by hydro-sulfite) | 55 |
| 1000 parts.                                                                   | 60 |

After hanging in the cold for about one hour, the goods are washed with water and developed at about 35° in a bath containing 20 parts of potassium persulfate and 37 parts of 66 Bé. sulfuric acid in 1000 parts of 65 water. Then they are washed and dried. Thereafter the wax is removed for instance by treating with benzine or benzene. The goods are advantageously again warm soaped and washed. In this manner white 70 effects on a violet groundation are obtained.

## Example 2

The dyed goods obtained according to Example 1 are printed after drying with any 75 pattern by means of a wax resist. Then they are treated in a cold bath prepared according to Example 1, but containing as sulfuric acid ester salt that of the dyestuff obtained according to Example 1 of U. S. Patent No. 1,504,584. Thereafter the goods are further treated according to Example 1. After removing the wax resist white and yellow effects are obtained on a groundation of a 80 violet shade and of a mixed shade of violet 85 and yellow.

## Example 3

A fabric containing wool or silk is dyed 90 in the customary manner light or middle

shades. The dried fabric is supplied with a wax resist and then dyed in the manner described in Example 1. The composition of shades thus obtained may be improved as regards their brightness by using for the previous dyeing a dischargeable dyestuff and adding to the second bath hydrosulfite (concentrated powder). Thereby instead of the mixed shades the pure shade of the dyestuff used for the cross dyeing is obtained.

*Example 4*

15 Wool or silk is dyed in the manner described in Example 1 with the employment of the ester salt of 6.6'-diethoxy-indigo, whereby white effects on orange are obtained. Then the goods are cross dyed with any wool 20 dyestuff. Besides the pure colored effect produced by the cross dyeing matter a mixed dyeing of both dyestuffs is obtained.

*Example 5*

25 Weighted or unweighted silk is treated according to Example 1 with a leuco-ester salt. The developing bath is replaced by a bath containing 1-2 parts of potassium chromate 30 and 18 parts of sulfuric acid in 1000 parts of water.

*Example 6*

35 Bleached wool or weighted or unweighted silk is printed on a cylinder printing machine provided with engraved heatable rollers with the following resist:

40 50 parts of beeswax,  
650 parts of colophony,  
30 parts of spermaceti,  
15 parts of molten mutton tallow,  
25 parts of paraffine,  
45 230 parts of oil of turpentine,  
1000 parts.

50 The goods are further treated according to Example 1.

*Example 7*

55 Self colored shades may be obtained by dyeing in the cold with leuco-ester salts according to Example 1 on a suitable piece dyeing machine or jigger and oxidizing as above described.

*Example 8*

60 Spun or woven dye goods (unweighted or weighted silk or chlorinated wool) are previously treated in a manner suitable for the printing process and advantageously printed 65 with a wax resist. Then they are treated

cold or lukewarm for one hour in the following bath:

10 parts of the sulfuric acid ester salt of leuco-6.6'-diethoxy-indigo, 70  
10 parts of formaldehyde-sulfoxylate,  
20 parts of triethanol-amine,  
960 parts of water,

1000 parts.

75 The dyeing is developed with one of the oxidizing baths mentioned in Examples 1 and 5.

*Example 9*

80 The process is carried out as described in Example 8, but the dye-path is replaced by the following one:

5 parts of the sulfuric acid ester salt of leuco-5.7.5'-trichloro-indigo, 85  
955 parts of water,  
10 parts of formaldehyde-sulfoxylate,  
20 parts of triethanol-amine,  
10 parts of sodium nitrite,

1000 parts.

90

The dyeing is developed in an acid bath whereto persulfate or chromate may be added.

I claim:

1. Process which comprises dyeing animal fibers in the cold with a bath containing sulfuric acid ester salts of leuco compounds of vat dyestuffs, an alkali of the group consisting of alkali metal carbonates and triethanolamine and reducing agents and developing the dyeing with a bath containing an acid and oxidizing agents of the group consisting of persulfate and chromate. 95

100 2. Process which comprises dyeing animal fibers, which are previously dyed and partially coated with a wax-resist, in the cold with a bath containing sulfuric acid ester salts of leuco compounds of vat dyestuffs, an alkali of the group consisting of alkali metal carbonates and triethanol-amine and formaldehyde sulfoxylate and developing the dyeing with a bath containing an acid and oxidizing agents of the group consisting of persulfate and chromate. 110

115 3. Process which comprises dyeing animal fibers, which are previously dyed and partially coated with a wax-resist, in the cold with a bath containing sulfuric acid ester salts of leuco compounds of vat dyestuffs, an alkali of the group consisting of alkali metal carbonates and triethanol-amine, reducing agents and nitrite and developing the dyeing with a bath containing an acid and oxidizing agents of the group consisting of persulfate and chromate. 120

125 In testimony whereof, I affix my signature.  
ALFRED FISCHESSER.

130